

1,426,623.

W. R. WEBSTER,  
METHOD OF MAKING BRASS AND SIMILAR ALLOYS,  
APPLICATION FILED MAR. 31, 1920.

Patented Aug. 22, 1922.



Inventor  
William R. Webster

By *Allyn B. Parsons*  
Attorney

# UNITED STATES PATENT OFFICE.

WILLIAM R. WEBSTER, OF BRIDGEPORT, CONNECTICUT.

## METHOD OF MAKING BRASS AND SIMILAR ALLOYS.

1,426,623.

Specification of Letters Patent. Patented Aug. 22, 1922.

Application filed March 31, 1920. Serial No. 370,221.

To all whom it may concern:

Be it known that I, WILLIAM R. WEBSTER, a citizen of the United States, residing in Bridgeport, county of Fairfield, and State 5 of Connecticut, have invented certain new and useful Improvements in Methods of Making Brass and Similar Alloys, of which the following is a full, clear, and exact description.

10 In making brass, the utilization of scrap is common practice, and in many cases the charge of metal introduced into the furnace for melting and subsequent casting contains a large percentage of scrap brass. For convenience in casting the brass ingots, the furnaces are preferably of the tilting type. The best results have been secured with tilting electric induction furnaces of the kind wherein a secondary consisting of a part of 15 the molten metal of the charge is located below the main body of the charge or bath, and is so arranged as to promote and maintain the circulation of the whole charge by motor effect. An efficient type of furnace 20 for the purpose in question is shown, for example, in the Clark Patent, No. 1,328,712, of January 20, 1920.

The development of the electric furnace has progressed to such a stage that the 25 proper temperatures for the melting of brass and similar scrap can be produced and maintained without difficulty. There has been difficulty, however, as regards the maintenance of a constant mixture,—that is to say, 30 a constant ratio of metals such as copper and zinc in the resulting product. This is due to the fact that the brass scrap available in the market has in its composition a varying and uncertain percentage of copper and 35 zinc. Where large amounts of this material 40 are melted in a brass furnace, considerable trouble is experienced in determining its composition by ordinary methods, because different portions of a particular lot or 45 quantity will have different compositions.

It is, of course, entirely possible to melt 50 such scrap in a furnace, draw a sample of molten metal from the furnace, and hold the charge molten in the furnace until the composition of the sample has been determined by chemical analysis. The necessary amount 55 of copper or zinc can then be added to the charge, so that the resultant mixture will be

what is desired. To make such a chemical analysis, however, requires in almost all 55 cases not less than half an hour, usually more. It will be understood, therefore, that, as furnaces employed for this work are capable of melting a charge in about one hour, the method just referred to (involving, if 60 practised the necessity for holding the furnace idle for about half the time, with the consequent loss of furnace capacity and expenditure of heat) is very expensive. This method is, in fact, so inconvenient and expensive that it is not employed under ordinary circumstances.

One of the primary objects of my invention is to overcome these drawbacks by providing a method whereby the composition of 70 the brass or similar alloy may be quickly but accurately determined, so that a constant mixture in the furnace product may be maintained in a commercially practicable manner.

Another object of the invention is to provide a method of producing castings of a uniform mixture from miscellaneous brass or other scrap without undue loss of furnace output.

To these and other ends, the invention consists in the novel features and procedure to be hereinafter described and claimed.

In the accompanying drawing, I have shown a hardness curve which may be used conveniently in the practice of my new 85 method.

It is well known that certain physical properties of brass and similar alloys vary with the percentages of the elements, e. g., copper and zinc, of which the alloy is composed. These physical properties or characteristics include tensile strength, percentage of elongation, hardness, electrical resistance, etc. I have found that by accurately determining the variation in physical 90 properties corresponding to varying percentages of copper and zinc in brass, for example, and expressing this relation in the form of a curve or table of corresponding values, it is possible by determining one of 95 the physical values of a brass of unknown composition, to determine its composition by reference to the above mentioned curve or table of values, and that by utilizing the information thus derived, in the manner hereinafter set forth, a valuable improvement in 100 105

the method of making brass and similar alloys may be obtained.

In carrying the invention into practice, my preferred procedure is as follows: 5 Samples of brass are procured, wherein the proportions of copper and zinc vary through a considerable range. These proportions are accurately determined by chemical analysis or otherwise. Samples are made or 10 procured, the compositions of which are say, successively 58 Cu, 42 Zn; 59 Cu, 41 Zn; 69 Cu, 40 Zn; 61 Cu, 39 Zn; 62 Cu, 38 Zn; etc. These samples are then tested in respect to one or more physical characteristics. 15 A suitable test for determining a physical value is furnished by a modification of the well-known Brinell hardness test. Brinell hardness is ordinarily measured by a number derived from the following:

20

$$\frac{L}{A} \times \sqrt[5]{R}$$

25 In this formula, L is the load in kilograms under which the ball is pressed into the material; A is the spherical area of the impression made by the ball, in square millimeters; and R is the radius of the ball, expressed in millimeters.

In the preferred practice of my invention, a steel ball of accurately known diameter is pressed into each sample by the application of a measured force as in the Brinell test; 30 but in order to save computation, a standard sized ball and a standard load are used in each instance, whereby a measurement of the impression of the ball gives all the information required. Preferably, the diameter of the impression is measured, and this can be done very accurately by the use of a micrometer microscope. A table is then prepared or a curve plotted, indicating the variation of the diameters of the impressions of the different samples, which diameters have been found to be proportionate to the copper content of the respective samples. The accompanying drawing shows such a curve where the abscissa represents, for example, the copper content, in per cent, and the ordinate represents, for example, the diameter of the ball impression in millimeters.

In manufacturing brass of a predetermined composition, where there is a fairly large percentage of scrap in the charge, I draw a sample from the molten charge and cool it. I then test it by the ball impression test and compare the result with the result 55 of the tests of the samples of accurately known composition, as shown, for instance, by the curve above mentioned. If, for example, the diameter of the impression in the sample unknown composition is 3.2, I find 60 the point where 3.2 lies on the ordinate of

the diagram and follow the horizontal line at that point to its intersection with the plotted curve. From this intersection I follow down the vertical line to determine the abscissa, which in this case will be 62 70 per cent. Knowing, therefore, that the copper content of the charge is 62 per cent, I then calculate from the weight of the entire charge, which has been previously determined, the amount of copper or zinc which 75 it is necessary to add to bring the charge to the desired composition, and such addition is then made.

The test preferred to can be made in approximately five minutes, and it will be 80 seen, therefore, that the practice of the invention overcomes the necessity of holding the furnace idle for a long period.

Another feature of great importance is the accuracy of determination which is possible by my new method in such a short time. 85 The composition of the alloy or mixture can be determined in most cases within one-half of one per cent of the exact figure, whereas in former ordinary commercial practice it 90 was difficult to keep the content of a given element within from three to four per cent of that desired.

Various changes may be made in the detailed procedure herein particularly described without departure from the scope 95 of my invention as defined in the claims.

In the preferred practice of the invention, owing to the fact that the electric furnace is not emptied completely when it is poured, 100 there is a certain residual charge, which tends to neutralize to a certain degree any variation in mixture in the succeeding charge. Also, the composition of the scrap can be predicted with considerable certainty in some cases, as where the scrap is being taken from a certain part of a car-load lot for example. Under these conditions, it will not be necessary to hold the charge molten in the furnace while a test is being made. 105 After casting a charge and making a test thereof in the manner previously described, the necessary correction in mixture can be made in the next charge and so on successively. On the other hand, there are numerous cases where the identification of the scrap is not at all good and where it is advisable to hold the charge while the test is being made and to change the composition of that particular charge, if necessary. It 110 is to be understood, therefore, that when reference is made herein to the addition to the charge in the furnace of sufficient copper or zinc to bring the material to the desired composition, this is not to be understood as 115 meaning the particular charge of which the test was made, but may refer to that or another charge.

Obviously, also, the improved method is applicable to the manufacture of alloys or 120

mixtures other than those containing copper and zinc, and if carried out in connection with the manufacture of brass, the same is applicable to a determination of the content 5 of metals other than copper and zinc, occurring either intentionally or as undesirable impurities.

What I claim is:

1. The method of making brass from 10 scrap, which comprises a determination of a value of a physical characteristic of each of a plurality of samples of brass having varying known proportions of copper and zinc, determining a comparable value of the same 15 physical characteristic of a sample of brass drawn from a molten furnace charge containing scrap brass, comparing those values to determine the composition of the last mentioned sample, and then adding to the charge 20 of metal in the furnace sufficient copper or zinc to bring the mixture to the composition desired.
2. The method of making brass or similar alloys, which comprises first ascertaining the 25 composition of the alloy while in the molten stage of its preparation, by determining the value of a physical property and comparing such value with those of similar alloys of known composition, and then in the light 30 of the obtained information, altering the molten alloy to obtain the desired composition.
3. The method of making brass and similar alloys, which comprises melting a charge 35 consisting at least partly of scrap metal, ascertaining the composition of the alloy while in the molten stage of its preparation by withdrawing a sample from the furnace, determining the value of a physical property 40 of such sample, and comparing such value with those of alloys of accurately known composition, and then in the light of the obtained information, altering the furnace charge to obtain the desired composition.
4. The method of making brass, where a 45 charge containing brass scrap is melted for casting, which comprises, first, a determination of the relative hardness of a number of brass samples of known composition having a successively increasing copper content, drawing a sample from the molten metal in the furnace, testing such sample for hardness, comparing the hardness of such sample with those of the above mentioned samples 55 to determine the relative composition of the sample drawn from the furnace, and then adding sufficient copper or zinc to the charge to bring the copper and zinc contents to the desired proportions.
5. The method of making brass, which 60 comprises melting in a suitable furnace a charge containing scrap brass, ascertaining the composition of the resulting alloy while in the molten stage of its preparation by 65 measuring the value of a physical property

thereof, and comparing such value with those of brass samples of accurately known composition, and then in the light of the obtained information altering the proportions of the furnace charge to obtain the desired 70 composition thereof.

6. The method of making brass or a similar alloy wherein a charge containing scrap is melted in a suitable furnace for subsequent casting, which comprises ascertaining the 75 composition of the furnace charge by withdrawing a sample of molten metal, permitting it to cool, measuring the value of a physical property of the sample, comparing such value with those of alloy samples of 80 accurately known composition, and then in the light of the obtained information altering the furnace charge so as to bring about the desired proportioning of the metals therein.

7. The method of making brass, wherein a charge containing brass scrap is melted in a furnace for casting, which comprises a determination of the hardness of a number of samples of brass of known, different composition by ball impression tests, plotting a curve in respect to said samples, drawing a sample from the molten metal in the furnace, testing it by ball impression to determine, by reference to the above mentioned hardness 90 curve, the percentage of copper in such sample, and then adding copper or zinc to the charge as required.

8. The method of controlling the composition of brass and similar alloys melted for 100 casting, which consists in determining values of a given physical property of a number of samples of known, varying contents, testing the material of unknown composition to determine the value of the same physical property thereof, comparing the value of such physical property with those of the above mentioned samples, and varying the composition of the casting charge as desired.

9. The method of controlling the composition of brass and similar alloys melted for casting, which consists in determining a given physical characteristic of a number of alloy samples of accurately known composition, said samples presenting a series having a successively increasing content of one metal, recording the variation in the value of such characteristic in the different samples, testing by a relatively rapid physical test the alloy of unknown composition to determine the value of the aforesaid physical characteristic thereof, comparing such value with the record of the corresponding values of the samples, and varying the casting charge to bring it to the desired composition.

10. The method of melting brass for casting, where at least a portion of the charge consists of scrap and where the charge is melted in a suitable furnace, which comprises the measurement of a given physical 130

characteristic of various samples of brass of accurately known but varying composition, recording such measurements as a series indicating a progressive increase in the content 5 of a given component of the alloy, testing a piece of metal which has been melted in the furnace so as to measure the aforesaid physical characteristic thereof and determine its relation to the series of samples in respect to 10 such physical characteristic, to determine thereby its relative composition, and then varying the charge in the furnace to bring it to the desired composition.

11. The method of melting brass for casting where the charge is melted in a furnace, which consists in testing by ball impression the hardness of a number of brass samples of known but varying composition having a progressively increasing content of one of 20 the metal components of the alloy, expressing and recording the hardness of such samples in a series, testing by ball impression the hardness of a brass piece of unknown composition which has been melted in the 25 furnace and has approximately the same temperature at which the samples were tested, and expressing such hardness in a comparable value, comparing such hardness value with the record of the varying hardness 30 of the samples so as to determine the composition of the piece of unknown composition, and thereafter varying the casting charge to bring it to the desired composition.

12. The method of melting metal for casting, where the charge is melted in a furnace, which consists in measuring a given physical characteristic of a metal of accurately known composition, drawing off from the molten metal in the furnace a sample of metal whose composition is to be determined, testing such sample to measure the aforesaid physical characteristic thereof in comparison with the metal of known composition, and adding to the furnace charge 40 the necessary material to bring the charge to the composition desired.

13. In the art of melting metal for casting, where a charge containing scrap metal is melted in a furnace, the method which 50 consists in determining a given physical property value of a number of metal samples of accurately known composition, testing when cold a piece of metal which has been melted in the furnace to ascertain the value 55 of the aforesaid physical characteristic thereof in comparison with the values of the metal samples previously mentioned, whereby the composition of the charge is determined, and then adding the necessary material to bring the charge to the composition desired.

14. In the art of melting metal for casting, the method which comprises determining the hardness values of a number of 60 metal samples of accurately known, differ-

ent composition, drawing off from the molten metal of the charge a sample, permitting the same to cool, then testing said sample for hardness and determining its hardness value in terms comparable to the first mentioned 70 hardness values, whereby the composition of the charge in the furnace may be ascertained, and then adding the necessary material to the charge to bring it to the desired composition.

15. In the art of melting metal for casting, where a charge containing scrap metal is melted in a furnace, the method which comprises a determination of the hardness values, by ball impression, of a number of 80 samples of accurately known, different composition, drawing off from the molten metal in the furnace a sample, permitting it to cool, testing it by ball impression to determine its hardness value and thereby its composition in relation to those of the samples of known composition previously mentioned, and then varying the composition of the 85 furnace charge as desired.

16. The method of melting metal for casting where the charge is melted in a furnace, which consists in testing by ball impression the hardness of a number of samples of known but varying composition, measuring the diameters of the impressions in the 95 various samples, recording such diameters in a progressive series, testing by ball impression the hardness of a piece of metal that has been melted in the furnace, measuring the diameter of the impression in such metal 100 piece so as to determine its place relatively to the series of samples and thereby its composition, and then varying the charge in the furnace to bring it to the desired composition.

17. In the art of melting metal for casting, the method which consists in determining the values of a given physical property of a number of metal samples of accurately known composition, testing when cold, by a 110 relatively rapid physical test, a piece of metal which has been melted in the furnace, to ascertain the value of the aforesaid physical characteristic thereof in comparison with the values of the samples, whereby the composition of such piece of metal is determined, and then varying the charge in the furnace to bring it to the desired composition.

18. The method of making brass and similar alloys, which comprises melting in a suitable furnace a charge consisting at least partly of scrap metal, ascertaining the composition of the alloy while in the molten stage of its preparation by withdrawing a 120 sample from the furnace, determining the hardness of the sample when cooled, comparing such hardness with those of alloy samples of accurately known composition, and then by the aid of the information 125 130

thereby obtained altering the molten alloy to obtain the desired composition thereof.

19. In the art of making alloys, the method of maintaining a constant mixture of metals in succeeding furnace charges, which consists in determining the values of a given physical characteristic of a number of alloy samples of accurately known but different composition, making a record of such values, testing from time to time a cooled piece of metal which has been melted in the furnace, to ascertain the comparable value of the aforesaid physical characteristic thereof, comparing such value with the aforesaid record so as to determine the composition of such piece of cooled metal, and then varying the charge as required to keep the mixture uniform.

20. In the manufacture of metallic alloys, where a charge containing scrap metal is melted in a furnace, the method of maintaining a substantially constant mixture in the furnace charge on repeated melting operations, which consists in determining the values of a given physical characteristic of a number of metal samples of similar alloys having accurately known but different composition, preparing a record of such values as a series, in which the content of one metallic component progressively increases, testing by a rapid physical test a cooled piece of metal which has been melted in the furnace, to ascertain the comparable value of its aforesaid physical characteristic, comparing such value with the aforesaid record to determine the composition of such cooled piece of metal, varying the furnace charge if necessary to bring it to the desired composition, and then repeating the test as above set forth from time to time in connection with different meltings, and varying the furnace charges to maintain a constant mixture in continued operation of the furnace.

21. In the art of making brass and similar alloys, the method which consists in ascertaining the composition of an alloy while in the molten stage of its preparation by measuring while the furnace is in operation the value of a physical property of a cooled piece of metal withdrawn from the bath, comparing such value with those of similar alloys of accurately known composition, and with the aid of the information thus obtained, altering the proportions of the constituents of the bath to obtain an alloy of the desired composition, and then pouring off a portion of the molten metal into a mold.

22. The method of making brass and similar alloys, where a charge containing scrap metal is melted for casting, which comprises a determination and recording of the relative values of one or more given physical characteristics of samples of a similar alloy having accurately known composition but successively increasing contents of one

metal, testing by a rapid physical test a cooled piece of metal which has been melted in the furnace, to ascertain in comparable terms the value of its aforesaid physical characteristic or characteristics, comparing such value with the record of the samples to determine the place of the tested piece in the series of samples and thereby the composition of the tested piece, varying the content of the furnace charge to bring it to a definite composition, and then repeating the test of a cooled piece of metal from time to time and comparing the result with the sample record, on different meltings, and varying the contents of the furnace charge as required to maintain an approximately constant mixture on repeated meltings.

23. In the art of making brass and similar alloys, where charges containing scrap metal are melted in a suitable furnace, the method which comprises ascertaining the composition of the alloy while molten in the furnace by determining the value of a physical property of a sample withdrawn from the furnace and cooled, comparing such value with those of similar alloys of accurately known composition, varying the furnace charge to bring it to the desired composition in the light of the information thus obtained, and then repeating the determination of the value of the said physical characteristic of cooled pieces of metal withdrawn from the furnace and the comparison thereof with the record from time to time and continuing the variation of the constituents of the furnace charge as required to maintain a substantially constant mixture in repeated operations.

24. In the art of making brass, where charges containing scrap metal are melted in a suitable furnace, the method of maintaining a substantially constant mixture in successive furnace charges, which comprises measuring the values of a given physical characteristic of a number of brass samples of accurately known composition, having different copper contents, preparing a record of such values, measuring from time to time the aforesaid physical characteristic of a piece of cooled metal which has been melted in the furnace, comparing such value with the record to determine the composition of such piece of cooled metal, and varying the contents of the charge, if necessary, subsequent to the tests so as to maintain a substantially constant mixture.

25. In the art of making brass, where charges containing scrap metal are melted in a suitable furnace, the steps of measuring and recording the values of a physical characteristic of a number of different brass samples of accurately known composition having successively increasing contents of copper, testing a cooled piece of metal which has been melted in the furnace to determine

the value of the aforesaid physical characteristic thereof and comparing it with the sample record, to ascertain the composition of such cooled piece of metal, varying the  
5 furnace charge to bring it to the desired composition, and then repeating the measurement of said physical characteristic of a cooled piece of metal and the comparison thereof with the record from time to time,

and varying the furnace charge as required 10 to maintain a substantially constant mixture.

In witness whereof, I have hereunto set my hand on the 19th day of March, 1920.

WILLIAM R. WEBSTER.

Witnesses:

M. A. TUTTLE,  
A. B. LYFORD.